

H. DAMAN,  
METHOD OF CASTING GLASS MOLDS,  
APPLICATION FILED NOV. 23, 1917.

1,295,277.

Patented Feb. 25, 1919.

FIG.1.



FIG.2.



WITNESSES

J. Herbert Bradley.  
Francis J. Domanson

INVENTOR

Herbert Damman  
by Christy and Christy  
his attorneys

# UNITED STATES PATENT OFFICE.

HERBERT DAMAN, OF ROCHESTER, PENNSYLVANIA.

## METHOD OF CASTING GLASS-MOLDS.

1,295,277.

Specification of Letters Patent. Patented Feb. 25, 1919.

Application filed November 23, 1917. Serial No. 203,509.

To all whom it may concern:

Be it known that I, HERBERT DAMAN, residing at Rochester, in the county of Beaver and State of Pennsylvania, a citizen of the 5 United States, have invented or discovered certain new and useful Improvements in Methods of Casting Glass-Molds, of which improvements the following is a specification.

10 The object of my invention is to provide a method of casting annular cast-iron glass-molds, whereby such molds will be rendered much more suitable and efficient for their intended purpose than are the molds as they 15 are now cast in actual practice.

My invention is predicated upon my discovery that by casting such glass-molds in molds, the inner and outer walls of which are formed of chill irons, the texture and 20 physical characteristics of the iron forming the glass-molds, and particularly the portion of the iron forming the interior surfaces of the glass-molds, are such that when the glass-molds are put in use the breakage 25 of the glass articles molded therein is much less than the breakage of such articles when molded in the glass-molds heretofore used, and furthermore that the articles molded therein have a superior surface.

30 While my invention is unlimited to glass-molds for any specific purpose, it finds particular adaptability to glass-molds used in pressing and blowing articles such as bottles, cans, etc. With respect to glass-molds for 35 such purposes, I have made the further discovery that, to obtain the best results, the outer chill iron of the casting mold should have a thickness of not less than about one fifth and not more than about one half of 40 the average wall thickness of the glass-mold.

My invention may be best understood by 45 describing it in detail with reference to the mold shown in the accompanying drawing, of which Figure 1 is a vertical central sectional view of the mold, and Fig. 2 a horizontal sectional view taken on the line II-II, Fig. 1. However, it will be understood that different specific forms of molds than that shown herein may be used in the 50 practice of my invention.

The shape of the glass-molds adapted to be cast in the mold shown herein is indicated by the cavity A. The mold comprises essentially an outer shell 1, preferably formed 55 of two parts as shown in Fig. 2, and a cen-

tral post or core 2. Both the shell and core are chill iron. Specifically, they are made of cast iron, and the thickness of the shell is not less than one fifth (preferably one third as indicated in the drawings) or more 60 than one half the average wall thickness of the glass mold cast between such shell and the core. The shell and core are preferably placed within a cheek 3, a cope 4 and a drag 5, all formed of sand and provided with 65 suitable casting sprues 6.

In casting a glass mold by means of the mold shown herein, the molten iron is poured into the sprues 6 in the usual manner until the cavity A is filled, the entrapped 70 gas and air escaping through the sand cope 4. When the iron solidifies, the casting is removed from the mold by separating the shell sections 1 and withdrawing the core 2. The glass-mold casting may then be ma- 75 chined in the usual manner.

The glass-mold thus cast is, as compared with the usual sand-cast glass-molds, dense, tough, and free from defects incident to graphitic carbon in large amounts; and the 80 surface is clean and smooth and not disfigured by objectionable hair cracks. As a consequence of these characteristics, I have found, as already stated, that when the glass-mold is put in use the breakage of the 85 glass articles molded therein is much reduced as compared to the breakage of such articles molded in the glass-molds heretofore used. These characteristics of the glass-mold I have found to be due to the 90 outer chill iron or shell 1. When such shell is omitted and the inner cavity of the glass-mold is formed by a cast-iron core 2, the resulting glass-mold does not have the above explained desirable characteristics. Fur- 95 thermore, I have found that such characteristics cannot be obtained, in glass-molds of the general shape shown herein, when the thickness of the chill iron or shell 1 is, as compared with the average thickness of 100 the glass-mold wall, otherwise than within the range already described.

I claim as my invention:

1. The herein described method of casting an annular cast-iron glass-mold, which 105 consists in forming the outer mold wall of a chill iron the thickness of which is not less than about one-fifth the average wall thickness of the glass-mold, forming the inner mold wall or core of a chill iron, and 110

casting the molten iron between said inner and outer chill irons.

2. The herein described method of casting an annular cast-iron glass-mold, which consists in forming the outer mold wall of a chill iron the thickness of which is not less than about one fifth and not more than about one half the average wall thickness of the glass-mold, forming the inner mold wall

or core of a chill iron, and casting the molten iron between said inner and outer chill irons.

In testimony whereof I have hereunto set my hand.

HERBERT DAMAN.

Witnesses:

JOSEPH M. EAKIN,  
S. A. ARMSTRONG.